

## UNITED STATES PATENT OFFICE.

HENRI TERRISSE AND MARCEL LÉVY, OF GENEVA, SWITZERLAND.

## ACID-PROOF CASTING.

No Drawing.

Application filed July 8, 1920. Serial No. 394,722.

*To all whom it may concern:*

Be it known that we, HENRI TERRISSE, a citizen of Switzerland, and MARCEL LÉVY, a subject of the King of Greece, residing at 5 Geneva, in the Confederation of Switzerland, have invented certain new and useful Improvements in Acid-Proof Castings, of which the following is a specification.

This invention relates to acid proof castings, and to a method or process of producing same.

It is a known fact that castings containing iron and silicon may be obtained, and that such castings will be proof against 15 mineral acids especially halogen acids, when said castings contain about 15 to 30 per cent of silicon. Such castings, however, cannot be easily made on account of the brittle nature of the mineral which will easily disintegrate and crumble to pieces. It is also known that ferro-tungsten and ferro-vanadium castings will also become acid-proof if a high percentage of tungsten or vanadium is used, but these alloys do not give 25 very satisfactory acid-proofness; and furthermore all such alloys of tungsten, vanadium or a mixture thereof are very difficult to cast.

We have found that all these disadvantages can be overcome, and that easily moulded castings which will have a very high resistance, either when cold or when warm, against halogen acids and other mineral or organic acids can be obtained. To 35 these ends, in accordance with the present invention, we make castings from mixtures of iron, silicon and a metal adapted to increase the mechanical and chemical resistance of the casting, such as, for example, tungsten, 40 or vanadium, or a mixture of the four metals.

In forming such castings, we subject ferro-silicon to heat to melt the same; and while in the molten state, we add thereto 45 at least one metal to increase its mechanical and chemical resistance, such metal being, for example, tungsten or vanadium.

These metals may be added either in a combined form, such as ferro-tungsten or 50 ferro-vanadium, or as the silicide of tungsten or silicide of vanadium.

In carrying out the process, iron and sili-

con are chosen so as to form ferro-silicon with from 10 to 30 per cent of silicon, so as to obtain an alloy having a melting point 55 at about 1200 to 1300° C. A metal such as ferro-tungsten or ferro-vanadium is then added thereto, so as to obtain an alloy containing from 2 to 20 per cent and more of tungsten or vanadium. 60

The castings thus produced will have great brightness and will not tarnish when exposed to the air and they will also have great acid-proofness and can be easily moulded. In analyzing such alloys, it has 65 been found that there will exist most probably some ternary combinations of iron, silicon and tungsten or of iron, silicon and vanadium, which combinations are very stable. 70

The ingredients may be used in about the following proportions:

*1st Example.*—100 kilograms of ferro-silicon having 20 per cent silicon are melted down, and 30 kilograms of ferro-tungsten 75 having 50 per cent tungsten are added thereto. The tungsten is rapidly dissolved in the molten metal and a homogeneous, easily running mass will be obtained. If a rapid chilling is desired, the casting is completed 80 by using chills.

*2nd Example.*—100 kilograms of ferro-silicon having 15 per cent silicon are melted down, and 28 kilograms of tungsten silicide having 19 per cent silicon are added thereto; the subsequent procedure being the same as in the first example. Ferro-vanadium and silicide of vanadium may be used instead of ferro-tungsten and silicide of tungsten. 9

We claim:

An acid proof casting which has great mechanical and chemical resistance made from an alloy containing iron, silicon, and tungsten, and which contains from ten to 9 thirty per cent silicon and from two to twenty per cent of tungsten.

In testimony whereof we affix our signatures in presence of two witnesses.

HENRI TERRISSE.  
MARCEL LÉVY.

Witnesses:

Dr. ROD. DE WURTEMBERG,  
THEODORE IMER.